

L. S. COPELIN.  
METHOD FOR RECOVERING VANADIUM.  
APPLICATION FILED MAY 28, 1920.

1,381,802.

Patented June 14, 1921.

*Fig. 1.*



*Fig. 2.*



*I. S. Copelin,*  
Inventor  
By *G. W. Metzger*,  
attorney

# UNITED STATES PATENT OFFICE.

LEONARD S. COPELIN, OF MILLERS, NEVADA.

## METHOD FOR RECOVERING VANADIUM.

1,381,802.

Specification of Letters Patent. Patented June 14, 1921.

Application filed May 28, 1920. Serial No. 384,923.

To all whom it may concern:

Be it known that I, LEONARD S. COPELIN, a citizen of the United States of America, residing at Millers, in the county of Esmeralda 5 and State of Nevada, have invented new and useful Improvements in Methods for Recovering Vanadium, of which the following is a specification.

The object of the invention is to provide 10 a simple, economical and inclusive method of recovering vanadium from ores and compounds including vanadium and particularly those which occur at normal temperatures in a solid form, under such conditions 15 as to obtain the vanadium in a form for commercial use at a cost which gives it a moderate commercial value.

In carrying out this object, it has been 20 found that sodium sulfid readily re-acts on vanadium compounds in the presence of steam and particularly when subjected to the action of heat and pressure and experiment has shown that under pressures of anywhere 25 from 5 to 250 pounds and at temperatures between 227 degrees F. and 406 degrees F. especially in the presence of steam, the reaction between the sodium sulfid and vanadium in the forms in which it occurs in ore, results in a resolution of the vanadium into 30 sodium vanadate which being soluble in water may be readily recovered and reduced by ordinary chemical means and methods in any suitable or preferred form for commercial use.

35 The experiments which have thus far been made in this connection, indicate that while the most suitable temperature to which to subject any particular ore containing vanadium must depend to a certain extent upon 40 the character of the ore, and therefore must be ascertained by experiment with the particular sample of the ore, the temperature which is valuable and will be found satisfactory in the large majority of instances is 45 in the neighborhood of 316 degrees F., while the pressure is about or near 70 pounds. In some instances, however, much lower pressures may be found practicable and even preferable and in other instances a much 50 higher pressure is desirable, and for corresponding reasons, the temperatures may vary both above and below that above indicated without losing the advantages which are incident to the exposure of the ore to 55 the combined effects of heat and pressure.

In carrying out the process it has been found desirable to employ apparatus such as that illustrated in the drawing wherein:

Figure 1, is a sectional view of a drum mounted for rotation and provided with a 60 steam jacket.

Fig. 2, is a view wherein the steam jacket is omitted.

The procedure which has been found efficient in this connection, is substantially as 65 follows:

Ground raw or roasted ore containing vanadium or solid vanadium compounds, and sodium sulfid in solution are placed in a drum such as that illustrated either in Figs. 70 1 or 2, or any equivalent container capable of withstanding a relatively high degree of heat and internal pressure. The amount of sodium sulfid in proportion to the ore or vanadium compound is not controlled by any particular rule or scale, and may be varied widely without in any way modifying the ultimate result of the process, the main desideratum being that the quantity of sodium sulfid— 75 with the additional water which may be employed, and which may be varied from 50% to 150% of the weight of the ore, shall be such as to make a pulp or mush which will be sufficiently soft and cohesive to pour. Obviously the amount of sulfur in the 80 sodium sulfid should be sufficient from a practical standpoint to combine with and absorb all of the materials which may be present in the ore such as lead, copper and zinc, and therefore the approximate amount 85 of sodium sulfid which may be used to the best advantage with any particular experiment on vanadium ore may readily be determined by experiment or by testing a 90 sample thereof.

Having placed the mixture as above indicated in the drum, the latter should be closed and the door or ground hole gap 10 thereof should be tightly secured so as to resist internal pressure, after which the drum should 100 be revolved to effect a thorough mixing or commingling of the ore and sodium sulfid to bring the particles of the former into contact with the latter.

The charge is now heated, as by the application 105 of steam either directly to the contents of the drum consisting as above indicated of the mixture of ore and sodium sulfid solution, or by introducing the same through tubes 11 or the equivalent thereof to the jacket 12, 110

2  
 steam pipes being carried into the drum through journals or trunnions 13 thereof which should be mounted in suitable bearings 14 to permit of imparting rotary movement to the drum. Obviously the heat introduced as above noted, either directly into the charge or into the steam jacket, will heat the charge and at the same time will produce an internal pressure in the drum by converting the sodium sulfid solution into steam and minute particles of sodium sulfid or steam incident to the vaporization of the water of the solution in which event the sodium sulfid solution will be highly concentrated. In either event the charge will be subjected to the combined action of heat and pressure in the presence of steam by which said heat and pressure are produced and with the sodium sulfid in intimate relation with the vanadium compounds and other minerals in the ore with the result that the sulfur of the sodium sulfid will replace the vanadium, while the vanadium will combine with the sodium of the sodium sulfid and take up oxygen from the minerals or other compounds under treatment or from the steam to form sodium vanadate. From two to four hours' time is required to effect a complete digestion of a charge of any substantial volume, and when the chemical re-actions have been completed, the drum may be cooled and the pressure reduced to normal to condense the steam, whereupon the vanadium will be found in the form of soluble sodium vanadate and will be in solution, which obviously may be readily separated from the solid matter or residue in the drum by filtration.

The vanadium may be recovered from the solution in any desired form by any preferred or well known chemical treatment, the reaction forming no part of the present invention.

The invention having been described, what is claimed as new and useful is:—

1. The method of recovering vanadium 45 from ores and compounds containing the same which consists in the treatment of the ore with sodium sulfid solution in the presence of heat.
2. The method of recovering vanadium 50 from ores and compounds containing the same which consists in the treatment of the ore with sodium sulfid solution in the presence of heat and under pressure.
3. The method of extracting vanadium 55 from ores and compounds including same which consists in the treatment of the ore with steam in the presence of sodium sulfid solution.
4. The method of extracting vanadium 60 from ores and compounds including same which consists in the treatment of the ore with steam in the presence of sodium sulfid solution and under pressure.
5. The method of extracting vanadium 65 from ores and compounds containing the same which consists in the treatment of the ores with sodium sulfid solution in the presence of steam while subject to heat and pressure.
6. The method of extracting vanadium 70 from ores and compounds including the same which consists in grinding ore and combining therewith a solution containing sodium sulfid to form a pulp and then subjecting the 75 mass to heat.
7. The method of extracting vanadium from ores and compounds containing the same, which consists in combining with the pulverized ore a solution containing sodium 80 sulfid and subjecting the mass to heat in a closed vessel.

In testimony whereof I affix my signature.  
 LEONARD S. COPELIN.